

Examiner  
of emulsion of thermoplastic  
materials, fillers  
and at least 30% 2,193,401  
of a aqueous solution of  
an inorganic salt for  
preproducing the composition  
and (a sodium silicate solution)

# UNITED STATES PATENT OFFICE

2,193,401

## SOUND DEADENING COMPOSITION

Benjamin Foster and Carl J. Seydel, Philadelphia,  
Pa., assignors to Benjamin Foster Company,  
Philadelphia, Pa., a corporation of Delaware

No Drawing. Application July 30, 1938,  
Serial No. 222,294

2 Claims. (Cl. 134—1)

This invention relates to methods of making, and to the products, sound deadening compositions that are also fireproof. The invention is particularly concerned with the methods of making, and the resulting products, of bituminous compounds which are used in sound and heat insulating installations.

The art of sound deadening and insulating metal vehicle bodies, such as automobile, train, airplane, and railway box cars, and the sound deadening and insulating of metal ventilating and air-conditioning ducts, metal wall partitions, metal doors, etc., has been highly developed in recent years. However, nearly all of the products used have serious objections which are due to the fire hazard present. This hazard exists because, either the sound deadener, or insulator itself, is not fireproof, or because the cement used to fasten a fireproof deadener in place on a structure is not fireproof.

This invention has for its objects to provide a sound deadening and fireproofing composition which may be applied to the surfaces of metal structures of all kinds, either as a plastic cement to be applied with a trowel, or sprayed upon the surface to be coated; or a suitable fabric such as burlap, or sheet asbestos, may be saturated with the composition, and the saturated sheet then secured to the surface to be coated by a layer of the plastic composition, and thereafter another layer of the plastic composition may be sprayed or otherwise applied to the installed saturated fabric sheet. Other methods of applying the plastic composition are described herein.

By "sound deadening" we mean the actual "deadening" of the tone emitted by a piece of metal, which of course has been set in vibration, and which has been treated by the application of some material applied for this purpose. This "deadening" effect is brought about, conventionally, by the application of a bituminous plastic material, or by cementing a piece of saturated or unsaturated roofing felt to the inside of the outside panel. The above method of deadening is most generally used on metal automobile bodies. In the case of a metal railroad coach or car a thick pad of hair felt is sometimes used. This is fastened in place with an asphalt adhesive. The effect of these materials is to lower the "natural" frequency of the vibrating panel, and to slightly decrease the total volume of sound emitted, and to act as a damper on the panel thereby shortening the duration of the sound.

As an illustration, a sheet steel panel about 20

inches by 20 inches by one-fourth inch thick, will normally vibrate at a frequency of about 140 cycles per second. Such a steel panel, uncoated, when set in vibration will continue to emit an audible tone for about 25 seconds, whereas after 5 coating with an efficient "sound deadening composition" will become silent in about 8 seconds; and in some cases, in a still shorter time. This shortening of the duration of the time of the sound is called the "decay time."

Again referring to the "bituminous plastic materials" which are extensively used, these compounds consist of an asphalt dissolved in a mineral or coal tar solvent, to which is added a filter or filters. The asphalts vary from low to 10 high softening points. The solvents vary from slow to quick drying volatile distillates. The filters vary in particle size and composition. There is generally, but not necessarily, asbestos fibre present, either alone, or in combination 20 with the other filters, which latter may be granulated cork, ground mica, ground charcoal, powdered mineral matter, for example talc or powdered sand, or a similar material. Another sound deadener, but one which is not so extensively used, consists of a clay type asphalt emulsion, either alone or pigmented with the filters described above, and in some cases weighted with a suitable grade of sand.

The plastic type of sound deadener described 30 above is generally applied in thicknesses of  $\frac{1}{8}$  inch to  $\frac{1}{4}$  inch, by using a spray gun made expressly for this purpose, or by brushing, or trowelling.

The objections to these types of products are 35 many, but the greatest one is the fact that none of them are fireproof. The solvent type sound deadener is easily burned either in the wet or dry state. The asphalt emulsion type of sound deadener is not easily burned in the wet state (it 40 is necessarily not combustible because of the water present) but is relatively easy to burn in the dry state.

The primary importance of a sound deadening material is "efficiency." This of course will 45 embody such requirements as: sound deadening value, fire resistance, ease of application, resistance to wear, adaptability to plant conditions such as (in the case of automobile bodies) baking, oil baths, alkali baths, etc. Of secondary 50 importance, but nearly as great as "efficiency" is "low cost". This not only refers to original cost per gallon, or pound, but also to the finished or applied unit cost. It is obvious that the more efficient a deadener per gallon or pound, the 55

smaller the quantity required to produce a desired effect.

The invention described herein meets all of the requirements outlined above, together with several other desirable characteristics. In the first place it is fireproof in both the wet and dry state. Also, when applied with the aid of an air gun the pressure required to force the compound from the pressure tank to the gun is in the neighborhood of 35 pounds per square inch, or less, as compared with the conventional 80 pounds per square inch minimum required for inflammable sound deadening compounds. With the new type there is no danger of explosions in the pressure tank, and practically no deteriorating action on the rubber hose which is used to supply the gun from the pressure tank.

It is common knowledge that bituminous materials such as asphalt, pitch, rosin, and resins, etc., are more or less waterproof. They are certainly insoluble in water. They are also thermoplastic. It is possible to prepare dispersions of these products in water, but no solution takes place. This particular art of dispersing bitumens in water is quite well covered by the prior art. It is not only impractical but impossible to dissolve the common inorganic salts in either asphalt or pitch. It is therefore not possible to take advantage of the fire resisting properties of these salts by any method known to date. We have discovered a method of incorporating certain inorganic salts with asphalt or pitch, and we obtain as a result a compound which is an excellent sound deadener, and also possesses the desired fireproof qualities.

In the manufacture of our sound deadening bituminous compound, several materials can be used, and as many or more ways of combining them. For example, we can first prepare a clay type bituminous emulsion consisting of approximately 40%-45% asphalt, 5%-7% clay, and 48%-55% water. To this prepared emulsion we can mix in approximately twice its weight of a solution of my water soluble fireproofing agent. This fireproofing agent can be a 50%-60% (or greater if so desired) solution of any of the following: sodium tungstate, ammonium-magnesium phosphate, sodium borate, boric acid, zinc chloride, calcium chloride, or sodium silicate. However, because of cost, we prefer to use a solution of sodium silicate. This is a commercial product and is commonly known as "water glass", "silicate of soda", and "sodium silicate." However, it is commercially available as a thick solution having varying gravities, and is designated as 40°-50°-60° etc. Baumé. In our composition we can use any of these grades depending upon the characteristics which we desire to impart to the product. After the addition of our fireproofing agent we can add to the mix a filler by simply stirring in, for example 15%-20% by weight of asbestos fibre and an equal quantity of granulated cork, or mica, or charcoal, or a similar material, or a suitable mixture thereof. If we so desire we can adjust the consistency of this finished product to enable it to be sprayed, brushed, or trowelled, simply by the addition of more fillers (if we desire it to be stiffer), or by the addition of the combined asphalt emulsion and fireproofing solution (if we desire it to be thinner).

Another example of how we can prepare the fireproof bituminous compound follows—we can prepare a clay type bituminous emulsion in the conventional manner and then add directly to this emulsion the fillers mentioned in the fore-

going example. These, of course, would be added in greater proportions, for example, 30%-40% asbestos, and 30%-40% of mica, ground cork, charcoal, etc., or a mixture thereof. The resultant mass will be a very stiff plastic. To this mass we can add my aqueous salt solution until we have obtained the proper consistency, or in such proportions as we desire.

A third example of how we have prepared the fireproof bituminous compound and which we can use if we so desire, but which should be used soon after preparation, consists of preparing an asphaltic cutback in the usual manner. That is by melting the asphalt and while still molten adding a volatile solvent to reduce the consistency to a 15 thick solution when cold, or at room temperature. We can also use any of the asphalt cutbacks which are commercially available. In either case, whether we prepare the cutback, or purchase it in its liquid form, we simply mix in the fillers which again consist of asbestos, mica, ground cork, charcoal, etc. The proportions are the same as given in the last example, namely, 30%-40% asbestos, and 30%-40% of the other materials. The resultant product is a heavy plastic 25 material. To this we simply add the aqueous salt solution and thoroughly mix it in. When making this type of compound it is necessary to add the preferred salt solution (silicate of soda) slowly, in order that no subsequent separation takes place. 30 The quantity of fireproofing agent will be approximately twice that of the combined cutback and fillers.

It is possible to make any or all of the described mixes by hand, that is, by stirring together the various materials; but it is desirable in commercial practice to use a power driven mixer. This mixer can be a paddle type horizontal or vertical device, or it can be the so-called "ribbon type" mixer. This latter type differs from the paddle 40 type only in that it has a series of ribbon-like arms fastened to the ends of the paddles. It is desirable to maintain a peripheral speed of from about 100 to 150 feet per minute when loaded.

In order to secure certain characteristics in the fireproof bituminous compound, we can vary the melting point and penetration of the asphalt used; or we can vary the grade of silicate of soda or other aqueous salt solution used. For example, if we desire a bituminous compound having a very 50 quick set and which, when dry, will be quite plastic, we can use a solution of sodium silicate having a Baumé gravity of say 40°, and an asphalt cutback or an asphalt emulsion prepared from a soft asphalt with a melting point of about 90°- 55 95° F. (ball and ring). If we desire the same setting time, and want the dried film to be quite hard, we can use a cutback or emulsion made from an asphalt having a melting point of about 190°-200° F. (ball and ring). If on the other 60 hand we desire a slow setting bituminous compound, we can use a solution of silicate of soda with a Baumé gravity of about 60°. By varying the melting point of the asphalt we can have the dried film either soft or hard, as we may choose. 65 Also it is possible to obtain combinations of these properties by using an asphalt with a melting point somewhere between 90°-200° F. (ball and ring), and a solution of silicate of soda having a Baumé gravity somewhere between 40°-60°.

The sound deadening composition prepared in any suitable manner, is a thick viscous mass at ordinary temperatures, and as noted above may be applied to a vertical surface to a thickness of as much as three-eighths of an inch without 75

flowing or sagging. During air drying, a "setting" occurs, the entire mass "self-welds" and hardens into an impervious and durable non-brittle layer. The asphalt or similar bitumen has the property of imparting a permanent adhesive or "wetting" property to dried inorganic salt films, for example, sodium silicate films, when the wet plastic is applied to a metal surface.

The prepared sound deadening compositions ready for application, may be applied at ordinary temperature, about 70 F. They may be applied to cold or hot (upwards to about 200° F.) metal surfaces. The compositions may contain ingredients in the following approximate proportions: in the asphalt cutback type, the asphalt may be present in from about 15% to about 20%; in the clay-asphalt-emulsion type, the emulsion may be present in from about 15% to about 30%. With both types, there may be about 15% of volatile solvent present. The filler, including asbestos, cork, talc, etc., may be present in from about 6% to about 10%. The aqueous solution of inorganic salt, for example, sodium silicate as described herein, may be present in from about 65% to about 70%. After air drying for a week or longer, the water content in the dried coating will be from about 5% to about 7%.

The improved sound deadening bituminous compounds described above exhibit properties which are quite foreign to previous bituminous admixes. For example, if any of them is applied to a piece of steel or other metal, it readily adheres to it even though it be in thickness of three-eighths inch or more. When freshly applied the compound can be subjected to the open flame of a Bunsen burner without showing any evidence of burning; the flame can be applied to either the coated or uncoated side of the metal. If this test is conducted on the conventional "cut-back type" deadener (which contains no aqueous salt solution), it immediately catches fire and burns if the flame is applied to the coated side of the metal. If the flame is applied to the under side or uncoated side, as soon as the solvent is slightly heated it flashes and burns.

When the uncoated side, or coated side, of a metal panel to which has been applied our improved sound deadening bituminous compound, is heated with a Bunsen burner flame the volatile solvent and the water are evaporated together and prevent the ignition of the said solvent. The silicate of soda or other salt then fuses and prevents the further vaporization of the asphalt. It is not our intent or purpose to heat a panel containing this compound to such a degree that the silicate of soda or other salt fuses; but in the event that sufficient heat be applied, this fusing

action will take place and prevent the ignition of the dried compound. When this fusing action has taken place the sound deadener coating no longer has its original sound deadening properties. One test, which demonstrates the fire resistance of the wet film, was conducted by spraying a one-fourth inch thick coat of the sound deadening bituminous compound upon a "19 gauge" cold rolled steel sheet, two feet square. While still wet, this panel was cut in two by using an oxy-acetylene flame. No burning of the compound was detected. It fused quite hard adjacent the cut but did not flame or burn. When the same test was conducted on the conventional "cutback" type sound deadener it was impossible to cut the sheet in half until all of the solvent and the asphalt had burned out of the mass. These tests, of course, are related here for the sole purpose of demonstrating the fire resistance of the new compound. However, there are occasions, during the manufacture of a bus, for example, where slight mechanical changes or repairs must be made shortly after the application of the sound deadener composition. When such changes necessitate the use of electric or gas welding, the possibility of serious fire damage is present when the conventional "cutback" type deadener is used. This fire hazard, as already pointed out, is not present when our improved sound deadening bituminous compound is used.

When our improved sound deadening bituminous compound is applied one-fourth inch in thickness upon metal, it can be either oven dried at temperatures up to 350° F. without sagging out of its original position, or without slipping or running or blistering. It also can be air dried and then subjected to temperatures of the order of 350° F. and still retain its original form. After either air drying or oven baking, it will withstand the same flame tests as the wet film. Air drying requires from 24 to 48 hours.

We claim:

1. A homogeneous sound deadening composition comprising from about 15% to about 30% of an aqueous clay type emulsion of thermoplastic bituminous material, from about 6% to about 40% of a filler, and not less than about 30% of an aqueous inorganic salt solution of substantially a 50% to about 60% concentration, said inorganic salt having fireproofing properties.

2. A sound deadening composition, as in claim 1, in which the aqueous inorganic salt solution is a solution of sodium silicate of about 40° to about 60° Bé., and is present in from about 50% to about 70%.

BENJAMIN FOSTER.  
CARL J. SEYDEL.